

## UNITED STATES PATENT OFFICE.

CHRISTIAN JOHN WERNLUND, OF TOTTENVILLE, NEW YORK, ASSIGNOR TO THE ROESSLER & HASSLACHER CHEMICAL COMPANY, OF NEW YORK, N. Y., A CORPORATION OF NEW YORK.

## METHOD AND ANODE FOR ELECTRODEPOSITION OF RUST-RESISTING COATINGS.

No Drawing. Original application filed January 5, 1924, Serial No. 684,506. Divided and this application filed July 6, 1925. Serial No. 41,867.

*To all whom it may concern:*

Be it known that I, CHRISTIAN JOHN WERNLUND, a citizen of the United States, and resident of Tottenville, in the county of 5 Richmond and State of New York, have invented certain new and useful Improvements in Methods and Anodes for Electrodeposition of Rust-Resisting Coatings, of which the following is a specification.

10 This invention relates in general to the electroplating on iron and steel or other metal articles of alloys with zinc of metals having a higher solution potential than iron, such as cadmium, this application being a division of my application, Serial No. 15 684,506 filed January 5, 1924.

Cadmium has many properties which render it advantageous over other metals and alloys as a protective coating for metals 20 such as iron and steel. It is light in color and has a higher solution potential than iron, thus tending to protect the iron from corrosion. As its solution potential is higher than that of iron and lower than 25 that of zinc, the same weight of protective coating of cadmium affords more protection to atmospheric corrosion than is offered by straight zinc. Also more cadmium than zinc can be deposited per unit of current 30 used. The oxide coating formed by atmospheric or other corrosion of cadmium is thinner and more adherent than that formed on zinc, consequently the tendency of cadmium to scale off and waste away is much 35 less pronounced than that of zinc.

While I have found that pure cadmium coatings can be effectively deposited electrolytically, I have further found that alloy coatings comprising cadmium retain in large 40 measure the advantages of pure cadmium coatings in durability and rapidity of deposit and can be much more cheaply and conveniently produced than previous coatings of pure cadmium. According 45 to my invention, I produce alloyed coatings comprising over 2% of cadmium and another metal, such as cadmium and mercury or zinc, or zinc, cadmium and mercury, using either plain anodes with a suitable bath, or alloy anodes, or both. The 50 coatings have the enhanced practical advantages characteristic of pure cadmium coatings in giving better protection than

zinc with less thickness, good color of coating, and economy of current. The advantage of using mercury in combination with cadmium or zinc and cadmium is that the resultant coating is more resistant to corrosion than cadmium or zinc alone. The cathode potential is raised with consequent 55 increased throwing power.

Such a coating may be formed by the use of a plating solution to which the proper addition of cadmium or cadmium and mercury compounds soluble in the bath have 60 been made, or the metals can be furnished to the solution by the use of cadmium anodes and zinc anodes or alloy anodes. If mercury is not desired in the final product 65 a binary anode of zinc and cadmium can be 70 used.

Examples of the scope of this invention are as follows:

*Example I.*

To plate steel casters with a zinc cadmium mercury alloy, they are cleaned by one of the alternative methods given in Example III depending upon their condition. When a chemically clean surface has been obtained 80 they may be plated in the following solution:

|                  |        |            |    |
|------------------|--------|------------|----|
| Water            | 1 L.   | 1 gal.     | 75 |
| Sodium cyanide   | 46 G.  | 6 oz.      | 85 |
| Sodium hydroxide | 30 G.  | 4 "        |    |
| Zinc cyanide     | 30 G.  | 4 "        |    |
| Cadmium hydrate  | 7.5 G. | 1 "        |    |
| Mercuric oxide   | 0.1 G. | 0.0125 oz. |    |

Other conditions maintained are as follows: 90

Temperature 40° C.  
E. M. F. 3 to 6 volts.  
Current 25 amperes per sq. ft.  
Anodes Zinc.

The bath must be replenished from time to time as the several ingredients become depleted. An average analysis of the coating obtained in zinc 70-80%, cadmium 20-30%, mercury 1-2%.

100

*Example II.*

I have also found that the zinc, cadmium and mercury contents of the bath may be stabilized by using zinc cadmium mercury 105 alloy anodes to supply the desired quan-

tities of these metals to the solution. A preferred composition of such an alloy anode is

|             | Per cent. |
|-------------|-----------|
| 5      Zinc | 73        |
| Cadmium     | 25        |
| Mercury     | 2         |

For some purposes, I have used a zinc cadmium mercury alloy anode of the following composition:

|             | Per cent. |
|-------------|-----------|
| 15     Zinc | 93        |
| Cadmium     | 5         |
| Mercury     | 2         |

15 to give a coating of approximately the same composition.

I do not claim specifically herein the novel products resulting from the processes and 20 baths herein disclosed, as such products are claimed in another application, Serial No. 684,507, filed January 5, 1924, patented Dec. 9, 1924, No. 1,518,622.

What I claim is:

25 1. Method of electrodepositing a rust resistant deposit of zinc, cadmium and mercury which consists in electrodepositing these metals from a solution of their salts in an aqueous sodium cyanide-sodium hydroxide solution.

30 2. Method of electrodepositing a rust resistant deposit of zinc, cadmium and mercury which consists in electrodepositing these metals from a solution of their salts in an aqueous sodium cyanide-sodium hydroxide solution wherein the article receiving the deposit is the cathode and an alloy of zinc, cadmium and mercury is the anode.

35 3. In cadmium electroplating from a cyanide bath, the step which consists in depositing cadmium in the presence of zinc and mercury to produce a coating of cadmium alloyed with zinc and a minor percentage of mercury.

40 4. In zinc electroplating from a cyanide bath, the step which consists in depositing zinc in the presence of cadmium and mercury to produce a coating of zinc alloyed with cadmium and a minor percentage of mercury.

45 5. In zinc electroplating from a cyanide bath, the step which consists in depositing zinc in the presence of a salt of cadmium

and of a salt of mercury capable of resisting reduction by the bath to produce a coating of zinc alloyed with minor percentage of cadmium and mercury.

55 6. Method of electrodepositing a cadmium alloy which consists in making the article to be plated the cathode and providing an anode whose major constituent is zinc the minor constituents being cadmium and mercury.

60 7. The method of electrodepositing an alloy coating of zinc and cadmium which consists in making the article to be plated the cathode and providing an anode whose major constituent is zinc and whose minor constituents are cadmium and mercury.

65 8. The method of electrodepositing an alloy coating of zinc cadmium and mercury which consists in making the article to be plated the cathode and providing an anode whose major constituent is zinc and whose minor constituents are about 5% of cadmium and about 2% of mercury.

70 9. The method of electrodepositing an alloy coating comprising cadmium from 2-30%, zinc from 70-97%, and mercury from 1-2% which consists in electrodepositing these metals from a solution of their salts in corresponding proportions in an aqueous sodium cyanide-sodium hydroxide solution.

75 10. The method of electrodepositing an alloy coating comprising cadmium from 2-30%, zinc from 70-97%, and mercury from 1-2% which consists in electrodepositing these metals from a solution of their salts derived from a ternary alloy anode of such metals in corresponding proportions in an aqueous sodium cyanide-sodium hydroxide solution.

80 11. An anode for electroplating comprising zinc cadmium and mercury in amounts effective for the purpose set forth.

85 12. An anode for electroplating comprising zinc, between 5 and 30% of cadmium, and about 2% of mercury.

90 13. An anode for electroplating comprising zinc, cadmium and mercury in which the mercury is in a smaller percentage than either the zinc or the cadmium.

95 Signed at Perth Amboy, in the county of Middlesex and State of New Jersey this 29th day of June A. D. 1925.

CHRISTIAN JOHN WERNLUND.